

# UNITED STATES PATENT OFFICE.

WILLIAM F. WENISCH, OF NEW YORK, ASSIGNOR TO HIMSELF AND JOHN WENISCH, OF NEWTON, N. Y.

## IMPROVED FIRE-KINDLING.

Specification forming part of Letters Patent No. **56,867**, dated July 31, 1866.

*To all whom it may concern:*

Be it known that I, WILLIAM F. WENISCH, of the city, county, and State of New York, have invented a new and useful Improvement in Composition for Lighting Fires; and I do hereby declare that the following is a full, clear, and exact description thereof, which will enable others skilled in the art to fully understand and make use of the same.

My invention has for its object to furnish an improved material to take the place of paper or shavings in starting wood or coal fires; and it consists of a composition for kindling fires, formed of the ingredients and prepared in the manner hereinafter described.

In preparing this composition I use rosin, dry sawdust, and dry sand, in the proportions of one pound of rosin, seven ounces of dry sawdust, and three ounces of dry sand. The rosin is put into an iron kettle and melted over a hot fire. The sawdust and sand are then mixed together in the above-mentioned proportions, and when the rosin is thoroughly melted the mixed sawdust and sand is poured in, and the mass is stirred and mixed until the ingredients are thoroughly intermingled. The composition is then taken out while hot and pressed in tin forms of any required shape.

I prefer to use shallow rectangular forms,

having ribs or low partitions across their bottoms, so as to partially divide the cakes into narrow rectangular blocks.

A part of one of these blocks about equal in amount to a cubic inch is sufficient to kindle a wood fire from two to three inches in thickness, and two or three times that amount will kindle a coal fire.

The tin forms should be greased occasionally, to prevent the composition from sticking fast to them when cold.

This composition can be readily lighted with a match, and does away entirely with any necessity for the use of paper or shavings in kindling fires.

I claim as new and desire to secure by Letters Patent—

A composition for kindling wood or coal fires, formed by combining rosin, dry sawdust, and dry sand with each other in the proportions and in the manner substantially as herein described, and for the purpose set forth.

The above specification of my invention signed by me this 25th day of May, 1866.

WILLIAM F. WENISCH.

Witnesses:

WM. F. McNAMARA,  
JAMES T. GRAHAM.